



US006258318B1

(12) **United States Patent**  
Lenczowski et al.

(10) **Patent No.:** US 6,258,318 B1  
(45) **Date of Patent:** Jul. 10, 2001

(54) **WELDABLE, CORROSION-RESISTANT  
AIMG ALLOYS, ESPECIALLY FOR  
MANUFACTURING MEANS OF  
TRANSPORTATION**

(75) Inventors: **Blanka Lenczowski**, Neubiberg;  
**Rainer Rauh**, Jetzendorf; **Dietrich  
Wieser**, Bonn; **Gerhard Tempus**,  
Bremen, all of (DE)

(73) Assignee: **EADS Deutschland GmbH**, Munich  
(DE)

(\*) Notice: Subject to any disclaimer, the term of this  
patent is extended or adjusted under 35  
U.S.C. 154(b) by 0 days.

(21) Appl. No.: **09/530,068**

(22) PCT Filed: **Aug. 14, 1999**

(86) PCT No.: **PCT/DE99/02549**

§ 371 Date: **Jun. 14, 2000**

§ 102(e) Date: **Jun. 14, 2000**

(87) PCT Pub. No.: **WO00/11229**

PCT Pub. Date: **Mar. 2, 2000**

(30) **Foreign Application Priority Data**

Aug. 21, 1998 (DE) ..... 198 38 017

(51) **Int. Cl. 7** ..... **C22C 21/06**

(52) **U.S. Cl.** ..... **420/542; 420/543**

(58) **Field of Search** ..... 420/542, 543

(56) **References Cited**

U.S. PATENT DOCUMENTS

4,645,543 2/1987 Watanabe et al. ..... 148/2  
5,624,632 4/1997 Baumann et al. ..... 420/544

FOREIGN PATENT DOCUMENTS

0918095 10/1993 (EP) .  
0563903 5/1999 (EP) .  
2717827 9/1995 (FR) .  
63-179040 7/1988 (JP) .

OTHER PUBLICATIONS

Patent Abstracts of Japan of JP 63-179040 Dated: Jul. 23,  
1998.

Brockhaus der Naturwissenschaften und der Technik, p. 161  
(1965) F.A. Brockhaus Wiesbaden.

Gschneider, Jr., K.A. "A critical Review of the Alloy Systems  
of the Rare Earth, Scandium and Yttrium Metals," in  
Rare Earth Alloys (1961) pp. XI & 12.

Filatov Y. A. "Weldable Aluminum-Magnesium-Scandium  
System Base Alloys" Welding in the World, Bd. 33, Nr. 6,  
(1994).

Database WPI Derwent Publications Ltd. XP002130336 &  
JP 52 011143 (Nippon Light Metal Res Lab) Jan. 27,  
(1977-01-27).

*Primary Examiner*—George Wyszomierski

*Assistant Examiner*—Janelle Combs-Morillo

(74) *Attorney, Agent, or Firm*—Ladas & Parry

(57) **ABSTRACT**

A weldable, corrosion resistant aluminum-magnesium alloy  
consisting essentially of 3 to 5% by weight magnesium  
(Mg), 0.05 to 0.15% by weight zirconium (Zr), 0.05 to  
0.12% by weight manganese (Mn), 0.01 to 0.2% by weight  
titanium (Ti), 0.05 to 0.5% by weight of one or more  
elements selected from the scandium group of the Periodic  
Table and/or terbium (Tb), wherein at least 0.15% by weight  
scandium (Sc) is included with or without terbium (Tb) and  
with or without 0.05 to 0.35% by weight of one or more  
elements from the lanthanide series, the balance being  
aluminum (Al), and unavoidable contaminants not exceeding  
0.2% by weight silicon (Si).

**7 Claims, No Drawings**

**WELDABLE, CORROSION-RESISTANT  
AlMg ALLOYS, ESPECIALLY FOR  
MANUFACTURING MEANS OF  
TRANSPORTATION**

**BACKGROUND OF THE INVENTION**

The invention relates to a weldable, corrosion-resistant, high-magnesium content aluminum-magnesium alloy, which contains a ternary aluminum-scandium-zirconium phase as an essential component. Such an alloy is disclosed in U.S. Pat. No. 5,624,632, for application in aerospace construction due to its low density, high strength and corrosion resistance. Adding rare earth or rare earth-like elements generates dispersoids in the aluminum-magnesium alloy, which produce a higher strength and corrosion resistance. The aforesaid U.S. patent is silent as regards the weldability of such an alloy.

**SUMMARY OF THE INVENTION**

An object of this invention is to provide a weldable, corrosion-resistant, high magnesium content aluminum-magnesium alloy, which is at least as good as the known alloy with respect to strength and corrosion resistance and exhibits a high recrystallization threshold and good weldability. This and further objects of the invention are achieved by a weldable, high magnesium-content aluminum-magnesium alloy consisting essentially of 3 to 5% by weight magnesium, 0.05 to 0.15% by weight zirconium, 0.05 to 0.12% by weight manganese, 0.01 to 0.2% by weight titanium, 0.05 to 0.5% by weight of at least one element selected from the scandium group of the Periodic Table, wherein scandium is present as a mandatory element optionally with terbium and/or 0.05% to 0.35% by weight of one or more elements in the lanthanide series, the balance being aluminum and unavoidable contaminants not exceeding 0.2% by weight silicon.

**DETAILED DESCRIPTION**

In comparison with the above described known alloy, in U.S. Pat. No. 5,624,632 the new alloy of the invention exhibits primarily a distinctly lower manganese content, whereby an improved corrosion resistance was surprisingly obtained, especially in a heat-treated state of parts made from this alloy, e.g., when cold-formed parts are subjected to an elevated temperature over a prolonged period of time. It was found that these positive properties are determined by the ratio of manganese to scandium. An improved corrosion resistance is found when the ratio of Mn to Sc is less than 2. Along with acting as a grain growth inhibitor, the titanium content (not present in the described known alloy) helps to

increase strength, since titanium can replace the zirconium in the ternary Al—Sc—Zr phase, wherein the solubility of titanium is lower than that of zirconium, however.

It has also been found that scandium can be replaced by terbium, at least within certain limits. However, more terbium than the amount of scandium being replaced must be added to achieve constant properties.

A particularly favorable alloy for motor vehicles ships and aircraft structures contains at least 0.15% by weight scandium. One or more elements from the Lanthanide series is preferably included in amounts ranging from 0.05 to 0.35% by weight. The alloy tolerates silicon contamination of up to 0.2% by weight, the dynamic properties of the alloy deteriorating above this level.

Although the invention is disclosed with reference to particular compositions, it will become apparent to those skilled in the art that numerous modifications and variations can be made which will fall within the scope and spirit of the invention as defined by the attached claims.

What is claimed is:

1. A weldable, aluminum-magnesium alloy comprising a ternary aluminum-scandium-zirconium phase and consisting essentially of 3 to 5% weight magnesium, 0.05 to 0.15% by weight zirconium, 0.05 to 0.12% by weight manganese, 0.01 to 0.2% by weight titanium, 0.05 to 0.5% by weight of at least one element from the group consisting of scandium and the lanthanide series, wherein at least scandium is present, the balance being aluminum, and unavoidable contaminants not exceeding 0.2% by weight silicon.

2. An aluminum-magnesium alloy as claimed in claim 1, wherein the ratio of manganese to scandium is less than 2.

3. An aluminum-magnesium alloy as claimed in claim 1, wherein at least 0.15% by weight of scandium is present in the alloy.

4. An aluminum-magnesium alloy as claimed in claim 1, wherein said at least one element from said group in addition to scandium comprises terbium.

5. An aluminum-magnesium alloy as claimed in claim 1, wherein said at least one element from the said group in addition to scandium is 0.05 to 0.35% by weight of an element in the lanthanide series.

6. An aluminum-magnesium alloy as claimed in claim 5, wherein said at least one element in the lanthanide series is neodyme, europium, gadolinium, dysprosium, holmium or erbium.

7. Rolled, extruded, welded or forged component of an aircraft, a ship or a motor vehicle consisting of an AlMg alloy according to claim 1.

\* \* \* \* \*

UNITED STATES PATENT AND TRADEMARK OFFICE  
**CERTIFICATE OF CORRECTION**

PATENT NO. : 6,258,318 B1  
DATED : July 10, 2001  
INVENTOR(S) : Blanka Lenczowski et al.

Page 1 of 1

It is certified that error appears in the above-identified patent and that said Letters Patent is hereby corrected as shown below:

Title page, Item [54] and Column 1, line 2,  
“AIMG” should read -- ALMG --.

Signed and Sealed this

Twenty-seventh Day of November, 2001

*Attest:*

*Nicholas P. Godici*

*Attesting Officer*

NICHOLAS P. GODICI  
*Acting Director of the United States Patent and Trademark Office*

UNITED STATES PATENT AND TRADEMARK OFFICE  
**CERTIFICATE OF CORRECTION**

PATENT NO. : 6,258,318 B1  
DATED : July 10, 2001  
INVENTOR(S) : Blanka Lenczowski et al.

Page 1 of 1

It is certified that error appears in the above-identified patent and that said Letters Patent is hereby corrected as shown below:

Title page.

Item [73], Assignee, after "(DE)" insert -- **Vaw Aluminium AG, Bonn (DE)** --.

Signed and Sealed this

Sixth Day of June, 2006



A handwritten signature in black ink, appearing to read "Jon W. Dudas". The signature is written in a cursive style with a large, stylized "J" at the beginning.

JON W. DUDAS  
*Director of the United States Patent and Trademark Office*